

## UNITED STATES PATENT OFFICE.

CARL LEYST, OF BERLIN, GERMANY, ASSIGNOR OF ONE-HALF TO ARTHUR HENRY LYMN, OF LONDON, ENGLAND.

## PROCESS FOR THE PRODUCTION OF CELLULOSIC MATERIAL.

No Drawing. Application filed November 11, 1926, Serial No. 147,849, and in Great Britain November 14, 1925.

This invention relates to a process for the production of cellulosic material.

Cellulose pulp is at present generally produced from wood, by one of three methods viz, 5 by the soda process, the sulphite process or by electric means, and from straw or grass such as esparto by the soda process only.

According to the soda process the wood, straw or grass is cut up into suitable size and 10 digested or boiled, strong alkali such as caustic soda liquor being run into the digester with the disintegrated raw material and cooked or boiled by the admission of steam for removing the incrustating substance from 15 the fibrous material.

After the boiling is complete the mixture of pulp and liquor is discharged into washing tanks where it is drained and freed from that coloured liquor the latter being evaporated 20 and treated for recovering the soda contained in it.

The washed pulp is thereafter screened, thickened and bleached or otherwise treated.

Now bamboo is a well known fibrous material which, if it could be treated economically, would be very suitable for the manufacture of cellulose pulp. However on account of the geographical situation of its growth this valuable material has not hitherto 30 been successfully commercially used for the production of cellulose.

It has already been proposed to boil crushed bamboo with water containing 5-25% lime, in order to obtain a paper makers half stuff, 35 but such a product is relatively voluminous and difficultly transportable, and so far as I am aware it has never been suggested to press the half stuff alleged to be obtained into a form suitable for cheap and economical transport.

The present invention however provides a simple and economical process for producing from bamboo an excellent cellulosic material adapted to be worked up into paper or the like 45 with a minimum additional expense, which process comprises finely disintegrating the bamboo, preferably by cutting the stems into pieces of a thickness of about one to five millimetres, boiling with quicklime until the 50 material can be worked up to a pulp and after washing the material thus obtained, forming it into cakes by submitting it to a moderate pressure which is adequate so that on sub-

sequent drying the cakes have obtained enough coherence to be transported. The 55 pulp cakes thus obtained can be further worked for example ground and treated with caustic soda of a low concentration when it is desired to convert the same into finished pulp, paper or the like.

In order to carry out the process successfully it is essential that the bamboo should be adequately disintegrated, as without this fine disintegration the subsequent action of the quicklime which softens the individual disintegrated particles so that they can be transformed into cake form, cannot be effected satisfactorily.

The lime boiling is carried out with about 35% by weight of quick-lime (based upon the dry bamboo material) in adequate water at a temperature of 95 to 100° C., and only for such a time until the material can be worked up to a pulp. This time is generally about ten hours. The lye is then removed and after 75 washing the pulp is milled with water.

The material thus obtained is then pressed into cakes which can be effected by hydraulic, mechanical or other means. The pressure for transforming the milled material into cakes 80 should be just sufficient to cause the cohesion of the cakes on subsequent drying. Any high pressure must be avoided because the subsequent disintegration of the cakes for further working up would be made too difficult.

The half stuff which has been obtained in this manner can be properly disincrustated by subsequent treatment with caustic soda of low concentration.

The pressed cakes of the present invention 90 take up comparatively small space which is a decided advantage in practice because the further working up of the bamboo pulp cakes can be effected at a place far away from the place where the material has been produced, 95 without necessitating excessive costs for transport. The present invention provides the further advantage that the after-treatment with caustic alkali required to convert the pulp cakes into finished pulp, paper or 100 the like can be effected with caustic soda of lower concentration than that usually required in paper manufacturing processes.

In order to understand the invention more clearly reference is made to the following 105 working example:—

The bamboo stems, about the thickness of an arm, from which the leaves have been removed, are cut to pieces on a sawing table and the knots removed. The internodal portions are placed in a squeezing press where they are sliced up and are thereupon disintegrated in a devilling machine, after which the material falls upon a transporter belt and is transferred by an elevator into a sile or boiler, preferably of the revolving type.

The bamboo, disintegrated to pieces of about 1 to 5 millimetres thickness and about 20 to 30 millimetres length, is introduced into a spherical iron boiler with about 35% by weight of quick-lime based upon the dry bamboo material and three times the amount of water and is heated by direct contact with steam to a temperature of 95 to 100° C., at which it is maintained for about ten hours. The lime is added in the form of milk of lime through a sieve of about 2 millimetres mesh adapted to retain as much as possible of the sandy residues. Every hour the boiler is revolved for about ten minutes in order to obtain a uniformly boiled product.

After the boiling has terminated, the lye is transferred to another boiler filled with bamboo. This procedure however cannot be repeated indefinitely as otherwise the colour and adaptability to bleaching of the final product is interfered with. After the removal of the lye, the boiler is filled with water two or three times and revolved and the water is discharged in order to wash out as much lime as possible from the boiled material. Finally the boiler is emptied and the bamboo, although freed only to a slight extent from its incrustations but loosened in structure and still containing about 60% moisture, is ground in a mill with addition of sufficient amounts of water until cake-formability has been attained (90 to 120 minutes) or until the chips have been opened up into fibres, which takes about 3 to 4 hours. The mass thus obtained which contains 75 to 80% water is pressed in a spindle press or hydraulic press with just sufficient pressure to cause coherence of the cakes when dried. After pressing, the cake still contains 50% water and has a fibre content of about 250 grs. per cubic decm. The cake thus obtained may either be air-dried or dried in a drying tunnel at 50 to 60° C., whereby the fibre content is increased to 300 grms. per cubic decm.

If the ground material is washed in known manner, prior to pressing, that is to say agitated with water and passed over a longitudinal sieve, the fibre content increases per unit volume from 15 to 18%.

In order to refine the material for the production of fine paper pulp or paper, the cakes are broken down and treated in the usual manner but with less than usual viz. 6 to 9% of caustic soda, (calculated on the dry bamboo material) in solution of adequate concentra-

tion. This treatment is carried out for about 4 hours at 2 atmospheres pressure and may be effected in the same spherical boilers in which the boiling with lime has been carried out. After the boiling is completed, the pressure is reduced, the waste lye removed, and the material left behind is conveyed to the bleaching apparatus. There it is concentrated and slowly (according to the degree of whiteness required) bleached by means of bleaching liquor of adequate concentration but containing 25 to 50% chloride of lime (calculated on the dry material) at 40° C. After the bleaching, the bleaching liquor is removed from the material which is again washed and thereupon worked on a cellulose pulp machine in the usual manner.

It has been found that when working with this process the following yields can be obtained:

By boiling the bamboo with lime the loss in the treatment lies between 6 and 8% and crushing entails a further loss of 9 to 10%. Thus in obtaining bamboo cake material, a yield of about 80 to 85% can be expected.

As previously stated the material may be improved by treating with caustic soda solution in order to render it easier to bleach. If this is done a loss of 16 to 20% occurs, so that a yield of only 60% is attained.

Bleaching the material entails a further loss of 5 to 15% according to the degree of bleaching. The yield of the improved and bleached material would then be about 45 to 50% of the original bamboo.

I claim:—

1. The process for the production of a cellulosic material suitable for use in paper manufacture, which comprises finely disintegrating bamboo, boiling the disintegrated bamboo with quick-lime to form a pulp, washing said pulp and rendering same coherent by compression.

2. The process for the production of a cellulosic material suitable for use in paper manufacture, which comprises finely disintegrating bamboo, boiling the disintegrated bamboo with quick-lime to form a pulp, washing said pulp, grinding the washed pulp and rendering same coherent by compression.

3. The process for the production of a cellulosic material suitable for use in paper manufacture, which comprises comminuting bamboo stems into pieces of an approximate thickness of about 1 to 5 millimetres, and suitable length, boiling the disintegrated bamboo with quick-lime to form a pulp, washing said pulp and rendering same coherent by compression.

4. The process for the production of a cellulosic material suitable for use in paper manufacture, which comprises comminuting bamboo stems into pieces of an approximate thickness of about 1 to 5 millimetres and

suitable length, boiling the disintegrated bamboo with quick-lime to form a pulp, washing said pulp, grinding the washed pulp and rendering same coherent by compression.

stems with about 35% by weight of quick-lime (based upon the dry bamboo material) in adequate water, at a temperature of 95 to 100° C., for about ten hours, removing the lye and washing the lime from the boiled material, thereupon treating the pulp thus obtained in a potcher with water for one and a half to two hours, submitting the mass thus obtained to sufficient pressure to form cakes, drying said cakes and treating same with soda lye. 70 75

5. The process for the production of a cel-  
lulosic material suitable for use in paper  
manufacture, which comprises cutting up  
bamboo stems into pieces of an approximate  
10 thickness of about 1 to 5 millimetres and  
suitable length, treating the cut bamboo  
stems with about 35% by weight of quick-  
lime (based upon the dry bamboo material)  
in adequate water, at a temperature of 95  
15 to 100° C., for about ten hours, removing the  
lye and washing the lime from the boiled  
material, thereupon treating the pulp thus  
obtained in a potcher with water for one and  
a half to two hours, submitting the mass thus  
20 obtained to sufficient pressure to form cakes  
and drying said cakes.

11. The process for the production of a cellulosic material suitable for use in paper manufacture, which comprises finely disintegrating bamboo, boiling the disintegrated bamboo with quick-lime to form a pulp, washing said pulp, rendering same coherent by compression, treating the compressed material with about 6 to 9% caustic soda (calculated on the dry material) in suitable solution in a boiler for about four hours at a pressure of about 2 atmospheres, removing the lye and washing the treated material with water, thereupon concentrating the pulp and treating same with 25 to 50% chloride of lime (calculated on the dry material) in adequate water at 40° C., finally washing the bleached material and working same on a cellulose pulp machine.

30 7. The process for the production of a cel-  
lulosic material suitable for use in paper  
manufacture, which comprises finely disinteg-  
rating bamboo, boiling the disintegrated  
bamboo with quick-lime to form a pulp,  
35 washing said pulp, grinding the washed  
pulp, rendering the ground material co-  
herent by compression and treating said com-  
pressed material with soda lye.

12. The process for the production of a 95  
cellulosic material suitable for use in paper  
manufacture, which comprises finely disinteg-  
rating bamboo, boiling the disintegrated  
bamboo with quick-lime to form a pulp, wash-  
ing said pulp, grinding the washed pulp, 100  
rendering the ground material coherent by  
compression, treating the compressed mate-  
rial with about 6 to 9% caustic soda (calcu-  
lated on the dry material) in suitable solu-  
tion in a boiler for about four hours at a 105  
pressure of about 2 atmospheres, removing the  
lye and washing the treated material with  
water, thereupon concentrating the pulp and  
treating same with 25 to 50% chloride of  
lime (calculated on the dry material) in ade- 110  
quate water at 40° C., finally washing the  
bleached material and working same on a  
cellulose pulp machine.

material with soda lye.

9. The process for the production of a cel-  
50 lulosic material suitable for use in paper  
manufacture, which comprises comminuting  
bamboo stems into pieces of an approximate  
thickness of about 1 to 5 millimetres and  
suitable length, boiling the disintegrated  
55 bamboo with quick-lime to form a pulp,  
washing said pulp, grinding the washed  
pulp, rendering the ground material coherent  
by compression and treating said com-  
pressed material with soda lye.

13. The process for the production of a cellulosic material suitable for use in paper manufacture, which comprises comminuting bamboo stems into pieces of an approximate thickness of about 1 to 5 millimetres and suitable length, boiling the disintegrated bamboo with quick-lime to form a pulp, washing said pulp, rendering same coherent by compression, treating the compressed material with about 6 to 9% caustic soda (calculated on the dry material) in suitable solution in a boiler for about four hours at a pressure of about 2 atmospheres, removing the lye and washing the treated material with water, thereupon concentrating the pulp and treating same with 25 to 50% chloride of lime (calculated on the dry material) in adequate 115 120 125 130

water at 40° C., finally washing the bleached material and working same on a cellulose pulp machine.

14. The process for the production of a cellulosic material suitable for use in paper manufacture, which comprises cutting up bamboo stems into pieces of an approximate thickness of about 1 to 5 millimetres and suitable length, treating the cut bamboo stems with about 35% by weight of quick-lime (based upon the dry bamboo material) in adequate water, at a temperature of 95 to 100° C., for about ten hours, removing the lye and washing the lime from the boiled material, thereupon treating the pulp thus obtained in a potsher with water for one and

a half to two hours and finally submitting the mass thus obtained to sufficient pressure to form cakes and drying said cakes, treating said cakes with about 6 to 9% caustic soda (calculated on the dry material) in suitable solution in a boiler for about four hours at a pressure of about 2 atmospheres, removing the lye and washing the treated material with water, thereupon concentrating the pulp and treating same with 25 to 50% chloride of lime (calculated on the dry material) in adequate water at 40° C., finally washing the bleached material and working same on a cellulose pulp machine.

20

25

30

In testimony whereof, I affix my signature.

CARL LEYST.